

## UNITED STATES PATENT OFFICE

2,549,737

## METHOD OF ELECTROPOISHING

Harold J. Wiesner, Elkhart, Ind., assignor to C. G. Conn, Ltd., Elkhart, Ind., a corporation of Indiana

No Drawing. Application July 19, 1946,  
Serial No. 684,796

3 Claims. (Cl. 204—140.5)

1

This invention relates to a method of and a bath for electropolishing and more particularly to the electropolishing of copper and copper alloys.

One of the objects of the invention is to provide a method of and bath for electropolishing in which all of the exposed surfaces of an article to be polished will be given a uniform bright finish free from discoloration.

Another object is to provide a method of and bath for electropolishing copper alloys containing lead which will produce a high luster free from smut.

The bath of this invention consists essentially of polyphosphates of the alkali metals and either borates or carbonates mixed therewith in an aqueous solution. The general formula covering this class of phosphates is



where M is a monovalent alkali metal and n is an integer equal to or greater than 3. The most satisfactory polyphosphates are those often referred to as the triphosphates or tripolyphosphates, the general formula being  $M_5P_3O_{10}$ .

It is to be understood that triphosphate and tripolyphosphate may be used interchangeably throughout this application. Sodium tripolyphosphate, for example, either as the pentahydrate or anhydrous salt may be used, or the corresponding potassium salts. These salts function in solution to form soluble compounds with the copper, zinc and lead and other metals commonly found in the copper base alloys during electropolishing. In the operation of the bath, the copper plates out as a sludge at the cathode after building up to a concentration of .05-.15 oz./gal. Thus, the net loss of tripolyphosphate is that which combines with the zinc, lead and other metals and that which is lost by drag-out. I have found that a satisfactory concentration is of the order of 12-16 oz. of a tripolyphosphate salt per gallon of solution although this concentration is not critical, and the bath will function satisfactorily with a concentration of tripolyphosphate as low as 8 ounces per gallon or up to its saturation point.

The effect of the borates and carbonates in the bath is to broaden the current density range and to obtain uniformity of polishing. If these materials are omitted there will be substantially less brightening in the recesses of the work and other low current density areas and etching may occur. Also, discolorations may occur in various areas of the work pieces. Among the specific compounds which I have found to be most satisfactory are boric acid, sodium tetraborate, potassium tetraborate, ammonium carbonate, sodium bicarbonate and potassium bicarbonate which are preferably used in concentrations of

2

from 2 to 12 ounces per gallon. If ammonium carbonate is used, it is necessary to keep the temperature of the bath below about 135° F. as above this temperature it decomposes rapidly. Ammonium carbonate and sodium and potassium bicarbonate also react with acid which may be added to the bath to lower its pH to give off some carbon dioxide. Boric acid and sodium or potassium tetraborate are preferred since they are thermally stable, do not decompose when acid is added and function to buffer the solution. While the ammonium radical is not in reality a metal, it will be identified hereinafter with sodium and potassium as the ion of an alkali metal.

In addition to these basic constituents of the bath, there may be added either an acid or a base in quantities sufficient to maintain the pH of the bath in the range from 7.0-8.5. For this purpose, sodium, potassium or ammonium hydroxide may be used to raise the pH. The sodium and potassium hydroxides are to be preferred as excessive amounts of ammonium salts are detrimental. For lowering the pH, tripolyphosphoric, metaphosphoric or orthophosphoric may be used.

If the pH is substantially below 7.0, the triphosphate hydrolyzes rapidly and the life of the bath is appreciably shortened. If on the other hand, the pH is substantially above about 8.5, the brightness of the electropolished surface diminishes.

The current density range may be further extended and greatly increased brightness produced by the addition of orthophosphate salts to the bath. Examples of satisfactory salts are sodium, ammonium or potassium salts such as mono, di or tri sodium or potassium phosphate and mono or di ammonium phosphate. The di sodium, di potassium and di ammonium phosphates, when put into solution, have pH values nearer to those in the operating range of the bath and for this reason are preferred. These salts when added to the bath in concentrations such that the  $PO_4^{3-}$  content is about 2.6-6.5 oz./gal. extend the current density range and greatly increase the brightness of the electropolished surface. The above mentioned concentrations correspond for example to about 10 to 24 oz./gal. of hydrated di sodium phosphate  $(Na_2HPO_4) \cdot 12H_2O$  or about 4.0 to 9.5 oz./gal. of anhydrous di sodium phosphate. This pronounced effect of the orthophosphate salts is particularly noticeable in the case of deeply recessed articles that are electro-polished.

In addition to the above mentioned functions, the salts of orthophosphoric acid also serve to buffer the solution. While their effect in broadening the current density and improving the brightness is not noted until a concentration of

about 4 oz./gal. of the anhydrous salt is attained, there will be an appreciable buffering effect well below this concentration. The salts may then be conveniently added at lower concentrations if it is desired only to obtain a more highly buffered solution.

It has further been found that the addition of oxalic acid or one of its salts such as sodium oxalate, ammonium oxalate or potassium oxalate in concentrations of about 4 to 6 ounces per gallon enables the temperature of the bath to be increased up to as much as 200° F. with good results. Without the addition of these materials, it has been found that the surface tends to become irregular at temperatures substantially in excess of 150° F.

In general, I have found that agitation of the work or of the solution during electropolishing is desirable. As a result of using agitation, higher current densities are permitted with less chance of "burning" the protruding sections of a complicated piece of work. The commonly employed methods of agitation used in the electroplating industry, such as oscillation of the work rod, air agitation, or solution agitation by means of pumps or paddles are satisfactory. The use of work rod oscillation is perhaps to be preferred.

The time required to polish to a high luster will vary with the particular material being polished and with the operating conditions. In general the time will vary from two to twenty minutes and will average about five to ten minutes.

In polishing according to the present invention the piece to be polished is connected as an anode in a bath constituted as described above and current is passed from the anode to a cathode which is preferably copper or plated with copper. The current density is preferably in excess of 100 amperes per square foot and may in some cases exceed 150 amperes per square foot. When so operated the pieces will be brought quickly to a uniform high luster without discoloration or smut.

As examples of baths which I have found satisfactory, the following may be given:

|                                      | Range         | Preferred               |
|--------------------------------------|---------------|-------------------------|
| EXAMPLE #4                           |               |                         |
| Sodium tripolyphosphate (anhydrous). | 8-saturation  | 14-16 oz./gal.          |
| Boric acid                           | 2-12 oz./gal. | 4-5 oz./gal.            |
| pH                                   | 7.0-8.5       | 7.0-7.5.                |
| Temperature, °F.                     | 100-212°      | 125-135°                |
| Current density                      |               | Above 100 amps./sq. ft. |

While the invention has been particularly described in connection with several specific bath compositions, it will be understood that various combinations and concentrations of the constituents mentioned as well as various operating conditions might be employed within the scope of the invention. The examples given are to be taken as illustrative only, reference being had to the appended claims for a determination of the scope of the invention.

What is claimed is:

1. The method of polishing copper and alloys in which copper is a major constituent which comprises connecting the alloy to be polished as an anode in an aqueous bath consisting essentially of a solution of a tripolyphosphate of an alkali metal and a material selected from the group consisting of boric acid, boric acid salts and salts of carbonic acid, said bath having a pH in the range from 7.0-8.5.

2. The method of polishing alloys in which copper is a major constituent which comprises connecting the alloy to be polished as an anode in an aqueous bath consisting essentially of a solution of a tripolyphosphate of an alkali metal and a material selected from the group consisting of boric acid, boric acid salts and salts of carbonic acid, maintaining the pH of the bath in the range from 7.0-8.5 and operating the bath at a temperature between 100° F. and 212° F. and at a current density in excess of 100 amperes per square foot.

3. The method of polishing alloys in which copper is a major constituent which comprises connecting the alloy to be polished as an anode in an aqueous bath consisting essentially of a solution of a tripolyphosphate of an alkali metal, a material selected from the group consisting of boric acid, boric acid salts and salts of carbonic acid and an orthophosphate salt and maintaining the pH of the bath in the range from 7.0-8.5.

HAROLD J. WIESNER.

#### REFERENCES CITED

The following references are of record in the file of this patent:

#### UNITED STATES PATENTS

| Number    | Name             | Date           |
|-----------|------------------|----------------|
| 2,086,867 | Hall             | July 13, 1937  |
| 2,226,384 | Norris           | Dec. 14, 1940  |
| 2,244,158 | Hubbard et al.   | June 3, 1941   |
| 2,294,227 | Delaplace et al. | Aug. 25, 1942  |
| 2,330,170 | Manuel           | Sept. 21, 1943 |
| 2,428,141 | Burkhardt        | Sept. 30, 1947 |

#### FOREIGN PATENTS

| Number  | Country       | Date           |
|---------|---------------|----------------|
| 435,710 | Great Britain | Sept. 26, 1935 |

|                                      | Range         | Preferred               |
|--------------------------------------|---------------|-------------------------|
| EXAMPLE #1                           |               |                         |
| Sodium tripolyphosphate (anhydrous). | 8-saturation  | 14-16 oz./gal.          |
| Boric acid                           | 2-12 oz./gal. | 4-5 oz./gal.            |
| pH                                   | 7.0-8.5       | 7.0-7.5.                |
| Temperature, °F.                     | 100-212°      | 120-140°                |
| Current density (average)            |               | Above 100 amps./sq. ft. |

|                            | Range         | Preferred               |
|----------------------------|---------------|-------------------------|
| EXAMPLE #2                 |               |                         |
| Potassium tripolyphosphate | 8-saturation  | 14-16 oz./gal.          |
| Boric acid                 | 2-12 oz./gal. | 4-5 oz./gal.            |
| pH                         | 7.0-8.5       | 7.0-7.5.                |
| Temperature, °F.           | 110-212°      | 120-140°                |
| Current density (average)  |               | Above 100 amps./sq. ft. |

|                                           | Range          | Preferred               |
|-------------------------------------------|----------------|-------------------------|
| EXAMPLE #3                                |                |                         |
| Sodium tripolyphosphate (anhydrous).      | 8-saturation   | 14-16 oz./gal.          |
| Boric acid                                | 2-12 oz./gal.  | 4-5 oz./gal.            |
| Di-sodium hydrogen phosphate (anhydrous). | 4-9.5 oz./gal. | 6.0-7.0.                |
| pH                                        | 7.0-8.5        | 7.0-7.5.                |
| Temperature, °F.                          | 110-212°       | 125-135°                |
| Current density (average)                 |                | Above 100 amps./sq. ft. |